

A. PRUESSMAN.  
MOISTURE PROOFING AND MOISTURE PROOFED TELEPHONE AND SWITCHBOARD  
CORD CONDUCTOR.  
APPLICATION FILED FEB. 16, 1912.

1,120,849.

Patented Dec. 15, 1914.

2 SHEETS-SHEET 1.



Witnesses.

Theo. R. George  
G. H. Johnson

Inventor:

Albert Pruessman

A. PRUESSMAN.

MOISTURE PROOFING AND MOISTURE PROOFED TELEPHONE AND SWITCHBOARD  
CORD CONDUCTOR.

APPLICATION FILED FEB. 16, 1912.

1,120,849.

Patented Dec. 15, 1914.

2 SHEETS—SHEET 2.



Witnesses:

*Thos. K. George  
A. H. Vorauer.*

Inventor:

*Albert Pruessman*

# UNITED STATES PATENT OFFICE.

ALBERT PRUESSMAN, OF CHICAGO, ILLINOIS, ASSIGNOR TO WESTERN ELECTRIC COMPANY, OF NEW YORK, N. Y., A CORPORATION OF ILLINOIS.

## MOISTURE-PROOFING AND MOISTURE-PROOFED TELEPHONE AND SWITCHBOARD CORD CONDUCTOR.

1,120,849.

Specification of Letters Patent. Patented Dec. 15, 1914.

Application filed February 16, 1912. Serial No. 678,029.

*To all whom it may concern:*

Be it known that I, ALBERT PRUESSMAN, citizen of the United States, residing at Chicago, in the county of Cook and State of Illinois, have invented a certain new and useful Improvement in Moisture-Proofing and Moisture-Proofed Telephone and Switchboard Cord Conductors, of which the following is a full, clear, concise, and exact 10 description.

This invention relates to insulated conductors, and more particularly to the application of waterproofing to flexible conducting cords.

15 The object of the invention is to impart moistureproof qualities to a fibrous covering of such conductors without impairing the electrical or mechanical efficiency of the conductor.

20 It is desirable in the manufacture of moistureproof conducting cords that the completed cord shall not show evidence of moistureproofing on the outer braidings as this would affect the appearance of the cord; 25 that it shall not expose any moistureproofing material as this would tend to interfere with the handling of the cord; that the moistureproofing shall not materially increase the dimensions of the cord and shall 30 not impart its flexibility, nor tend to exert any deteriorating effect upon materials used, and that the insulation resistance shall be materially improved, particularly when the cord is used in humid atmosphere.

35 In accordance with this invention, the conductor, which may be a plurality of assembled tinsel strands, is first covered with one or more layers of fibrous insulating material. The conductor thus covered is 40 drawn through a heated insulating compound at a rate of progression permitting saturation of the outer portion of the fibrous covering but without permitting penetration sufficient to coat the conductor itself or 45 saturate the strands thereof. Preferably, the fibrous covering consists of two independent helical layers reversely wound, and the conductor is passed through the insulating compound at such speed that the outer

50 layer is completely and the inner layer but partially saturated. A blast of cold air may be applied to the conductor after it emerges from the tank and before it is wound on the reel, in order to cool the compound and pre-

vent the turns of the conductor from sticking together. 55

The accompanying drawings show a convenient arrangement of apparatus for practising the method indicated in a commercial manner. 60

Figure 1 is a view in elevation of a suitable tank with means for advancing the conductor and for heating the insulating compound; Fig. 2 is a continuation of the view shown in Fig. 1 and includes a winding reel 65 and a polishing die; Fig. 3 is a sectional view of a flexible conducting cord; and Fig. 4 is a view of a finished, flexible, conducting cord, such as is used in the telephone service.

The tank *t* is supplied with a waterproofing compound which may consist of asphaltum 91%, resin 6%, and resin oil 3%. The compound in the tank is heated as uniformly as possible by gas jets *b*. Near one end of the tank there is a fixed vertical sieve or 70 screen *s*, the object being to allow no foreign matter to appear in the liquid material or to come in contact with the conductors. There is a reel *r* rotatably supported on an axle *a*; a friction brake *d* is applied to the axle to 75 vary its freedom of rotation. There is a rotating device, like *e*, for agitating the liquid, and at each end of the tank are sliding frames *f* carrying grooved rollers *g*; a conductor *c* is passed back and forth over these 80 rollers and drawn in over a roller *h* and out over a similar roller *h'*; it then passes through smoothing dies *i* and *j* and through a heated polishing die *k*, which is rapidly 85 rotated, and is then wound on a reel *v*. The conductor *c* is composed of a plurality of strands of tinsel shown at 10 in Fig. 3; on 90 this is a braiding of tinsel strands 11, and on this are one or more layers 12, 13, of reversely wound fibrous insulating material. 95 such as silk or wool. The moisture-proof insulating material is represented at 14. This permeates the layers 13 and just enters the layer 12 without coming in contact with the conductor 10, 11. Outside the moisture-proof material 14, applied as described, is a 100 finishing covering of braided insulating material like 15.

The temperature of the compound in the tank *t* should be maintained at from 390° 105 to 420° Fahrenheit. The compound is heated to a minimum working temperature of 390° Fahrenheit in order that it may be

- thinned to a point necessary for properly impregnating the conductor, and is kept from exceeding a maximum of 420° Fahrenheit to avoid injuring the conductor by over-heating. A good specimen of conductor is insulated with double tussah floss, or with single worsted; such a conductor is passed through the tank in six lengths or passes, immersing from sixteen to twenty four feet 10 of conductor in the compound. It requires one minute to properly impregnate the double tussah floss insulated conductor and fifteen seconds to insulate the wool covered conductor. Under these conditions the comparative outputs are respectively 1440 feet per hour for the tussah floss and 3840 feet per hour for the wool insulated conductor. The insulating compound, when the conductor is passed through the tank at the rate of 20 3840 feet per hour, will cool, under ordinary conditions, within a distance of twelve feet after leaving the tank; but as it is desirable to cool it as quickly as possible in order to prevent the turns of the conductor from sticking together, a blast of cold air should be applied to the conductor by some suitable means such as an electric fan shown at *w* in Fig. 2 after it emerges from the tank and before it is wound on the reel.
- 80 What I claim and desire to secure by Letters Patent is:
1. The process of rendering a flexible conductor, consisting of a plurality of tinsel strands, moisture proof and retaining the flexibility thereof, which consists in applying thereto an inner and an outer layer of fibrous insulating material and drawing said insulated conductor through a heated insulating compound at a rate of progression permitting saturation of said outer layer 40 and of the outer surface of said inner layer.
  2. The process of rendering a flexible conductor moistureproof and retaining the flexibility thereof, which consists in applying thereto an inner and an outer layer of 45 fibrous insulating material, saturating said outer layer with insulating compound, and permeating only the outer surface of said inner layer with said compound.
  3. The process of rendering a flexible conductor moistureproof and retaining the flexibility thereof, which consists in applying thereto a covering of fibrous insulating material and drawing such insulated conductor through a heated insulating compound at a rate of progression permitting the saturation of said insulating material to a depth less than the thickness thereof. 50
  4. In a flexible conducting cord, the combination of a conducting core, an inner and an outer layer of fibrous insulating material forming a covering therefor and an insulating compound saturating said outer layer and the outer surface of said inner layer. 60
  5. In a flexible conducting cord, the combination of a conducting core, a fibrous covering therefor, and an insulating compound saturating said fibrous covering to a depth less than the thickness thereof. 65

In witness whereof, I, hereunto subscribe 70 my name this 6th day of February A. D., 1912.

ALBERT PRUESSMAN.

Witnesses:

THEO. R. GEORGE,  
A. H. VOMM.